

1

3,748,091

PROCESS FOR DYEING POLYESTER TEXTILES  
David Melville Fawkes, Manchester, England, assignor to  
Imperial Chemical Industries Limited, London, England

No Drawing. Filed Apr. 7, 1971, Ser. No. 132,183  
Claims priority, application Great Britain, Apr. 22, 1970,  
19,288/70

Int. Cl. D06p 1/20

U.S. Cl. 8—39

6 Claims

## ABSTRACT OF THE DISCLOSURE

Process for dyeing or optically brightening cellulose triacetate and aromatic polyester textile materials which comprises treating said textile materials with a dispersion of a dyestuff or optically brightening agent which contains at least one optionally substituted carbonamido or sulphonamido group in a halogenated hydrocarbon and in the presence of a small amount of water, the said treatment being carried out at a temperature above the boiling point of the azeotrope of the halogenated hydrocarbon and the water, and at a pressure above atmospheric pressure.

This invention relates to an improved process for the dyeing or optical brightening of cellulose triacetate and aromatic polyester textile materials and their blends with other textile materials.

It has previously been proposed to dye or optically brighten synthetic textile materials at elevated temperatures with solutions or dispersions of water-insoluble dyestuffs or optically brightening agents in a chlorinated hydrocarbon solvent, especially perchloroethylene, optionally containing small amounts of water, the said treatment being optionally carried out at pressure above atmospheric pressure. This process suffers from the disadvantage that the affinity of the said dyestuffs or optically brightening agents is low, so that only pale shades can be achieved by this process.

It has now been found that a particularly valuable class of dyestuffs or optically brightening agents which can be used are those which are insoluble or only slightly soluble in the chlorinated hydrocarbon and which contain at least one optionally substituted carbonamido ( $-\text{CONH}_2$ ) or sulphonamido ( $-\text{SO}_2\text{NH}_2$ ) group as, under these particular methods of application, this class of dyestuffs or optically brightening agents has a much higher affinity for synthetic textile materials.

According to the present invention there is provided an improved process for dyeing or optically brightening cellulose triacetate and aromatic polyester textile materials which comprises treating said textile materials with a dispersion of a dyestuff or optically brightening agent which contains at least one optionally substituted carbonamido or sulphonamido group in a halogenated hydrocarbon and in the presence of a small amount of water, the said treatment being carried out at a temperature above the boiling point of the azeotrope of the halogenated hydrocarbon and the water, and at a pressure above atmospheric pressure.

The process of the invention can be conveniently carried out by immersing the textile material in a dispersion of the said dyestuff or optical brightening agent in the halogenated hydrocarbon containing the necessary amount of water, which mixture is preferably contained in an autoclave or other pressure vessel, sealing the autoclave and thereafter heating it for a period which usually does not exceed 2 hours to a temperature above the boiling point of the azeotrope of the halogenated hydrocarbon and the water. At the conclusion of the process the dyed or optically brightened textile material may be rinsed with the

2

halogenated hydrocarbon solvent or some other solvent such as acetone to remove excess dyebath liquor and/or unfixed dyestuff, and the textile material is then dried. However in order to remove all unfixed dyestuff from the surface of the textile material, in particular polyester textile materials, it is preferred to give the dyed textile material a treatment in a clearing bath comprising an emulsion of an aqueous alkaline solution of sodium hydrosulphite in perchloroethylene.

The amount of water present in the dyeing process is preferably between 0.2% and 5% based on the volume of the halogenated hydrocarbon.

Although the dyeing process is carried out at a temperature above the boiling point of the azeotrope of the halogenated hydrocarbon and the water, it is preferred that the temperature be equal to or greater than the boiling point of the pure halogenated hydrocarbon.

As examples of halogenated hydrocarbons which can be used in the process of the invention either singly or in the form of mixtures there may be mentioned chloroform, carbon tetrachloride, dibromoethylene, trichloroethylene, 1:1:2-trichloro-1:2:2-trifluoroethane, 1:1:1-trichloroethane, and preferably tetrachloroethylene, (perchloroethylene).

There can also be present emulsifying agents which can be anionic, cationic or non-ionic. Non-ionic emulsifying agents may be, for example (a) polyethers of hydroxy, mercapto and amino compounds such as polyalkoxy-fatty alcohols, polyalkoxy polyols, polyalkoxy-mercaptans, polyalkoxy-aliphatic amines, polyalkoxy-alkylphenols, polyalkoxy-naphthols, polyalkoxyalkylarylmercaptans and polyalkoxyalkylarylamines, (b) fatty acid esters of ethylene glycol, polyethyleneglycols, propyleneglycols, butene-glycols, glycerine, polyglycerine, pentaerythritol and sugar alcohols such as sorbitol, sorbitan and saccharose, (c) N-hydroxyalkylcarbonamides, polyalkoxycarbonamides and polyalkoxysulphonamides. Anionic emulsifying agents may be for example of the classes of alkylsulphonates, alkylarylsulphonates, alkylsulphates, aliphatic carboxylates and mono- or di-alkyl esters of phosphoric acid. Cationic surfactants may be for example quaternary ammonium salts. Specific examples of such classes of emulsifying agents are to be found in "Solubilisation by Surface Active Agents" by Elworthy, Florence and Macfarlane, published by Chapman and Hall Ltd., in 1968.

The dyestuffs and optical brightening agents which can be used in the process of the invention can be of any of the recognised classes of dyestuffs, for example, methine, styryl, phthalocyanine, phthaloperinone, quinphthalone, azo, anthraquinone and nitro dyestuffs, and optical brightening agents, for example stilbenes, coumarins, pyrazolines, naphthalimides, carbostyryls, 1:3:4-oxodiazoles, 1:3:4-thiadiazoles, ox(thio- or imido-)azoles having fused aromatic rings, and heterocyclic derivatives of polycyclic hydrocarbons such as 2:4-dimethoxy-1:3:5-triazin-6-yl pyrene and 4-(2':4':dichloro-1':3':5'-triazin-6'-yl)-1-methoxynaphthalene, which are free from sulphonic acid groups and which contain at least one optionally substituted carbonamido or sulphonamido group each of which is directly attached to a carbon atom of an aryl radical present in the molecule of the dyestuff or the optically brightening agent or is attached thereto through an alkyne or an alkyleneamino radical. Such groups can be conveniently represented by the formula:



wherein X represents  $-\text{CO}-$  or  $-\text{SO}_2-$ , and  $\text{R}^1$  and  $\text{R}^2$  each independently represent a hydrogen atom or an optionally substituted alkyl, cycloalkyl, aryl or heterocyclic radical, or  $\text{R}^1$  and  $\text{R}^2$  are joined together to form with

the nitrogen atom N a 5- or 6-membered nitrogen-containing heterocyclic ring.

As examples of the radicals represented by R<sup>1</sup> and R<sup>2</sup> there are mentioned lower alkyl such as methyl, ethyl, propyl and butyl, substituted lower alkyl for example hydroxy lower alkyl such as  $\beta$ -hydroxyethyl, lower alkoxy lower alkyl such as  $\beta$ -methoxyethyl and  $\gamma$ -methoxypropyl, cyano lower alkyl such as  $\beta$ -cyanoethyl, aryl substituted lower alkyl such as benzyl, cyclohexyl, optionally substituted phenyl such as phenyl itself and tolyl, anisyl, chlorophenyl and bromophenyl.

As examples of the 5- and 6-membered nitrogen-containing heterocyclic rings formed by joining together R<sup>1</sup>, R<sup>2</sup> and the nitrogen atom N there may be mentioned pyrrolidine, indoline, piperidine, morpholine, piperazine and N-alkylpiperazine.

It is however preferred that R<sup>1</sup> and R<sup>2</sup> each represent a hydrogen atom.

The said dyestuffs and optical brightening agents can themselves be obtained by any of the conventional methods of producing dyestuffs and optical brightening agents from intermediates containing the said carbonamide or sulphonamide groups or by directly introducing such groups into the preformed compounds. Typical methods include, for example:

(a) Treating a dyestuff or optical brightening agent with chlorosulphonic acid and reacting the resulting sulphonchloride with the appropriate amine.

(b) Reacting a dyestuff or optical brightening agent containing a carboxylic acid group or groups with thionyl chloride and treating the resulting acid chloride with the appropriate amine.

| Example | Amine                                                  | Coupling component                                      | Shade            |
|---------|--------------------------------------------------------|---------------------------------------------------------|------------------|
| 2       | 4-aminobenzene sulphonamide                            | N:N-di( $\beta$ -hydroxyethyl)aniline                   | Yellowish-orange |
| 3       | do                                                     | N-methyl-N-( $\beta$ -hydroxyethyl)aniline              | Do.              |
| 4       | do                                                     | N-methyl-N-( $\beta$ -cyanoethyl)aniline                | Yellow           |
| 5       | do                                                     | N-ethyl-N-( $\beta$ ; $\gamma$ -dihydroxypropyl)aniline | Yellowish-orange |
| 6       | 4-aminobenzene carbonamide                             | N:N-di( $\beta$ -hydroxyethyl)-m-toluidine              | Do.              |
| 7       | 4-aminobenzene sulphon-N-( $\beta$ -hydroxyethyl)amide | do                                                      | Do.              |
| 8       | 2-chloro-4-nitroaniline                                | 3-sulphonamido-N:N-di( $\beta$ -hydroxyethyl)aniline    | Bluish-red       |

(c) Reacting together intermediates which give a dyestuff or optical brightening agent (for example a diazo component and a coupling component) at least one of which contains a carbonamide or sulphonamido group.

The dispersion of the dyestuff or optical brightening agent in the halogenated hydrocarbon can be conveniently obtained by milling or grinding the dyestuff or optical brightening agent in the halogenated hydrocarbon in the presence of a deflocculating agent. As deflocculating agents there may be mentioned, for example, polyureas which are essentially free from basic amino groups and which contain at least two urea groups and at least two groups each of which is an alkyl, alkenyl or alkaphenyl group containing at least eight carbon atoms, and which are soluble in organic solvents.

The cellulose triacetate and aromatic polyester, especially polyethyleneterephthalate, textile materials can be in the form of fibres or filaments or knitted or woven goods. If desired the said textile materials can be in the form of blends with other textile materials particularly cotton and woollen textile materials.

When applied to synthetic textile materials by the process of the invention the said dyestuffs and optical brightening agents have excellent affinity thus enabling heavy depths of shades to be obtained, and the resulting dyed or optically brightened textile materials have excellent fastness to the tests commonly applied to such textile materials.

The invention is illustrated but not limited by the following examples in which the parts and percentages are by weight:

#### EXAMPLE 1

0.2 part of the monoazo dyestuff obtained by coupling diazotised 4-aminobenzenesulphonamide with N-ethyl-N-( $\beta$ -hydroxyethyl)aniline is dispersed by milling in 800

parts of perchloroethylene in the presence of 0.1 part, as deflocculating agent, of the polyurea product prepared as described below. 2 parts of water are added, the mixture is placed in a dyeing vessel and 20 parts of polyethylene terephthalate textile material in the form of staple cloth is immersed in the mixture. The dyeing vessel is then sealed and heated at 120° C., for 30 minutes to effect dyeing. The dyed textile material is then removed from the pressure vessel, rinsed in acetone to remove the excess dyebath liquor and any loosely bound dyestuff, and is finally dried. The textile material is thereby coloured a deep yellowish-orange shade of excellent fastness properties.

The polyurea product used in the above example was itself obtained as follows:

A solution of 73.7 parts of a commercially available 40% solution in butyl acetate of polymerised mixed 2:4- and 2:6-tolylene diisocyanates containing 5.7% of isocyanate groups and less than 0.5% of free tolylene diisocyanate in 32 parts of acetone was added to a stirred solution of 53.5 parts of a fatty secondary amine derived from soya and commercially available under the trade name Armeen 25 ("Armeen" is a registered trademark) in 118 parts of acetone at 50° to 55° C. The acetone was then removed by distillation under reduced pressure.

In place of the dyestuff used in Example 1 there are used the monoazo dyestuffs obtained by diazotising the amines listed in the second column of the following table and coupling the resulting diazo components with the coupling components listed in the third column of the table. The fourth column of the table lists the shades of the resulting dyeings.

| Example | Amine                                                  | Coupling component                                      | Shade            |
|---------|--------------------------------------------------------|---------------------------------------------------------|------------------|
| 2       | 4-aminobenzene sulphonamide                            | N:N-di( $\beta$ -hydroxyethyl)aniline                   | Yellowish-orange |
| 3       | do                                                     | N-methyl-N-( $\beta$ -hydroxyethyl)aniline              | Do.              |
| 4       | do                                                     | N-methyl-N-( $\beta$ -cyanoethyl)aniline                | Yellow           |
| 5       | do                                                     | N-ethyl-N-( $\beta$ ; $\gamma$ -dihydroxypropyl)aniline | Yellowish-orange |
| 6       | 4-aminobenzene carbonamide                             | N:N-di( $\beta$ -hydroxyethyl)-m-toluidine              | Do.              |
| 7       | 4-aminobenzene sulphon-N-( $\beta$ -hydroxyethyl)amide | do                                                      | Do.              |
| 8       | 2-chloro-4-nitroaniline                                | 3-sulphonamido-N:N-di( $\beta$ -hydroxyethyl)aniline    | Bluish-red       |

#### EXAMPLE 9

0.1 part of the monoazo dyestuff obtained by coupling diazotised 4-aminobenzenesulphonamide with N:N-di( $\beta$ -cyanoethyl)aniline is dispersed by milling in 320 parts of perchloroethylene containing 0.05 part of the polyurea obtained as described in Example 1 above. 2 parts of water are then added, and the resulting mixture placed in a dyeing vessel. 20 parts of a polyester fibre which is commercially available under the trade name of Crimplene ("Crimplene" is a registered trademark) are then immersed in the mixture, the dyeing vessel is sealed, and dyeing then carried out for 30 minutes at 130° C. The dyed textile material is then removed from the vessel, rinsed in acetone to remove excess dyebath liquor and any loosely bound dyestuff, and is then dried. A deep yellow shade of excellent fastness properties is thereby obtained.

#### EXAMPLE 10

In place of the dyestuff used in Example 9 there is used 0.1 part of the monoazo dyestuff obtained by coupling diazotised 3-chloro-4-aminobenzenesulphonamide with N-methyl-N-( $\beta$ -cyanoethyl)aniline, and the dyeing is then carried out for 30 minutes at 120° C. A deep orange dyeing of excellent fastness properties is obtained.

#### EXAMPLE 11

0.1 part of the dyestuff obtained by coupling diazotised 4-aminobenzenesulphonamide with N-methyl-N-( $\beta$ -cyanoethyl)aniline is dispersed in 320 parts of perchloroethylene containing 0.05 part of the polyurea described in Example 1. 2 parts of water are added, the mixture placed in a dyeing vessel and 20 parts of cellulose triacetate fabric are immersed in the liquid. The vessel is sealed and dyeing carried out for 30 minutes at 95° C. The dyed material is then removed from the dyebath, rinsed in aqueous ethanol,

and is dried. A deep yellow shade of excellent fastness properties is obtained.

The following table gives further examples which illustrate the invention, the dyestuff used in Example 10 being replaced by the dyestuffs obtained by diazotising the amines listed in the second column of the table and coupling with the coupling components listed in the third column of the table. The fourth column of the table gives the shades of the resulting dyeings.

wherein X represents  $-\text{SO}_2-$  and  $\text{R}^1$  and  $\text{R}^2$  each independently represent hydrogen, lower alkyl, hydroxy lower alkyl, lower alkoxy lower alkyl or cyano lower alkyl in a halogenated hydrocarbon and in the presence of between 0.2% and 5% water based on the volume of the halogenated hydrocarbon, said treatment being carried out at a temperature above the boiling point of the azeotrope of the halogenated hydrocarbon and the water, and at a pressure above atmospheric pressure.

| Example | Amine                                                         | Coupling component                                           | Shade                        |
|---------|---------------------------------------------------------------|--------------------------------------------------------------|------------------------------|
| 12      | 4-aminobenzenesulphonamide                                    | 1-ethyl-3-cyano-4-methyl-6-hydroxypyrid-2-one                | Greenish-yellow.             |
| 13      | do                                                            | N-methyl-N-( $\beta$ -cyanoethyl)-m-toluidine                | Orange.                      |
| 14      | 3-nitro-4-aminobenzenesulphonamide                            | N-methyl-N-( $\beta$ -cyanoethyl)aniline                     | Do.                          |
| 15      | 4-aminobenzenesulphon-N-( $\beta$ -chloroethyl)amide          | N:N-di( $\beta$ -cyanoethyl)aniline                          | Yellow.                      |
| 16      | 3-chloro-4-aminobenzenesulphon-N-( $\beta$ -chloroethyl)amide | do                                                           | Do.                          |
| 17      | 2-amino-5-nitrobenzamide                                      | do                                                           | Red.                         |
| 18      | do                                                            | N-methyl-N-( $\beta$ -cyanoethyl)aniline                     | Red.                         |
| 19      | 2-aminobenzothiazole-6-sulphonamide                           | do                                                           | Red.                         |
| 20      | do                                                            | N:N-di( $\beta$ -cyanoethyl)aniline                          | Red.                         |
| 21      | do                                                            | N-ethyl-N-( $\beta$ -cyanoethyl)-m-toluidine                 | Violet.                      |
| 22      | 2-amino-5-nitrobenzenesulphon-N-methylamide                   | N-methyl-N-( $\beta$ -cyanoethyl)aniline                     | Red.                         |
| 23      | do                                                            | N:N-di( $\beta$ -cyanoethyl)aniline                          | Red.                         |
| 24      | 4-nitroaniline                                                | 2-naphthylamine-3-sulphonamide                               | Red.                         |
| 25      | 2-chloro-4-nitroaniline                                       | do                                                           | Red.                         |
| 26      | 2-cyano-4-nitroaniline                                        | 2-naphthylamine-4-sulphonamide                               | Bluish-red.                  |
| 27      | 2-chloro-4-nitroaniline                                       | 2-naphthylamine-4-sulphon-N-( $\beta$ -hydroxyethyl)amide    | Reddish-viol <sup>a</sup> t. |
| 28      | do                                                            | N-ethyl-N-( $\beta$ -carbamoylethyl)aniline                  | Violet.                      |
| 29      | 4-methoxyaniline                                              | N-ethyl-N-( $\beta$ -carbamoylethyl)aniline                  | Orange.                      |
| 30      | 2-carboxy-4-nitroaniline                                      | N-methyl-N-( $\beta$ -carbamoylethyl)aniline                 | Violet.                      |
| 31      | 2-methylsulphonyl-4-nitroaniline                              | do                                                           | Bluish-red.                  |
| 32      | 2-cyano-4-nitroaniline                                        | do                                                           | Do.                          |
| 33      | do                                                            | 3-acetylamo-N-methyl-N-( $\beta$ -carbamoylethyl)aniline     | Bluish-viol <sup>a</sup> t.  |
| 34      | 2-amino-5-nitrothiazole                                       | N-( $\beta$ -cyanoethyl)-N-( $\beta$ -carbamoylethyl)aniline | Blue.                        |
| 35      | 2-aminobenzothiazole-6-methylsulphone                         | N-ethyl-N-( $\beta$ -carbamoylethyl)-m-toluidine             | Red.                         |
| 36      | 4-nitroaniline                                                | N-methyl-N-( $\beta$ -sulphamoylethyl)aniline                | Red.                         |
| 37      | do                                                            | N-ethyl-N-( $\beta$ -sulphamoylethyl)-m-toluidine            | Bluish-red.                  |
| 38      | 2-cyano-4-nitroaniline                                        | do                                                           | Violet.                      |
| 39      | 2,4-dinitro-6-bromoaniline                                    | 2-ethoxy-5-acetylamino-N-( $\beta$ -sulphamoylethyl)aniline  | Blue.                        |

#### EXAMPLE 40

In place of the 0.1 part of dyestuff used in Example 10 there is used 0.1 part of 1:4-diaminoanthraquinone-2-carbonamide or of 1:4-diaminoanthraquinone-2-carbo-N:N-di( $\beta$ -hydroxyethyl)amide or of 1-amino-4-( $\beta$ -hydroxyaniline)anthraquinone-2-carbonamide whereby reddish-blue, reddish-blue and blue dyeings respectively are obtained of excellent fastness properties.

#### EXAMPLE 41

0.01 part of the fluorescent brightening agent 1:4-di-(4-carbamoylstyryl)benzene is milled in 320 parts of perchloroethylene containing 0.005 part of the polyurea described in Example 1. 2 parts of water are added, the mixture placed in a dyeing vessel, 20 parts of an aromatic polyester fabric are added, the vessel sealed and then heated for 30 minutes at 120° C. The fabric is then removed from the vessel, rinsed in perchloroethylene and dried. The fabric is brighter than the untreated fabric.

#### EXAMPLE 42

The procedure of any of the above examples is repeated but there is additionally incorporated into the dyebath liquor 0.4 part of isopropylammonium dodecyl benzene sulphonate (which is an emulsifying agent commercially available under the trade name of Arylan PWS) whereby similar results are obtained.

I claim:

1. A process for dyeing or optically brightening aromatic polyester textile materials which comprises treating said textile materials with a dispersion of a dyestuff or an optically brightening agent which contains a sulphonamido group of the formula



2. Process as claimed in claim 1 wherein the halogenated hydrocarbon is perchloroethylene.

3. Process as claimed in claim 1 wherein the dispersion contains a deflocculating agent.

4. Process as claimed in claim 1 wherein the dispersion contains an emulsifying agent.

5. Process as claimed in claim 1 wherein the dyestuff is an azo dyestuff which contains at least one unsubstituted sulphonamido group directly attached to a carbon atom of an aryl radical or attached thereto through an alkylene or alkyleneamino radical.

6. Process as claimed in claim 1 wherein the dyestuff is an anthraquinone dyestuff which contains at least one unsubstituted sulphonamido group directly attached to a carbon atom of an aryl radical or attached thereto through an alkylene or alkyleneamino radical.

#### References Cited

##### UNITED STATES PATENTS

- 3,622,558 11/1971 Koller et al. 8-50 X  
 3,623,834 11/1971 Seuret et al. 8-62 X  
 2,725,390 11/1955 Fogelman et al. 8-173 X  
 3,623,833 11/1971 Wildermuth et al. 8-40

##### FOREIGN PATENTS

- 1,192,984 5/1970 Great Britain 8-174  
 1,535,352 6/1968 France 8-174

##### OTHER REFERENCES

Ciba-Geigy Review, 1971/4, pp. 11-13.

65 LEON D. ROSDOL, Primary Examiner

T. J. HERBERT, JR., Assistant Examiner

U.S. Cl. X.R.

8-41 C, 174